

Aug. 23, 1932.

E. WIEGAND

1,873,730

ELECTRON EMITTING MATERIAL

Filed Oct. 2, 1928



INVENTOR  
ERICH WIEGAND

BY *W. G. Moore*

ATTORNEY

## UNITED STATES PATENT OFFICE

ERICH WIEGAND, OF HOHEN NEUENDORF, GERMANY, ASSIGNOR TO ALLGEMEINE ELEKTRICITATZ GESELLSCHAFT, OF BERLIN, GERMANY, A CORPORATION OF GERMANY

## ELECTRON EMITTING MATERIAL

Application filed October 2, 1928, Serial No. 309,892, and in Germany November 2, 1927.

In the production of discharge tubes, with or without rare gas filling, such as receiver or transmitter tubes for wireless telegraphy, rectifier tubes and the like, the metals of the 5 alkaline earths are customarily employed for many purposes. They are employed for instance for the production of highly emitting oxide cathodes, in that they are developed in the form of vapor in the tubes, are then 10 deposited on a carrier body and there, for instance, converted into oxide, after having been alloyed with the metal of the carrier body through conversion with substances giving off oxygen.

15 They are further employed for improving vacuum and also, on account of their low cathode fall, as electrodes in discharge tubes of the most various kinds. Since the metals of the alkaline earths are very base, it is very 20 difficult to get them into the tubes, without their being sharply attacked and becoming ineffective. For this reason only certain 25 combinations of alkaline earths recently have been employed in practice, to wit, the acids and specifically, the salts of the nitrogen-hydrogen acids, which are constant, in the air at ordinary temperature, but which, at higher 30 temperatures, decompose, forming metal of alkaline earth. This process has, however, disadvantages, which interfere considerably with its utility.

Apart from the high price of the acids and their explosiveness, which render the accumulation of great quantities of the same at one 35 point inadvisable, above all other considerations, the fact carries weight, that the pumping time of the tubes is very considerably prolonged by the great quantities of gas (nitrogen) freed by the decomposition of the acids.

40 Furthermore, the output of metal is comparatively small, since, on decomposition, in addition to metals, other alkaline earth combinations are formed in great quantities. Thus from barium acid, for instance, up to 45 75% of barium nitride results. A very particular disturbance in connection with the use of tubes of this kind, is the deterioration of the vacuum, which occurs for no apparent reason and which renders the utility of the 50 tubes questionable.

Now it has been found, contrary to the general expectation, that the reason for this phenomenon is to be sought in the process of the generation of the alkaline earth metal from acid. If now, in contradistinction to this process, the metal is produced in the tube in such a way that certain alkaline earth combinations evolving no gases at the glow temperature, such as oxides, aluminates etc. are heated with reducing agents which do not noticeably volatilize at the converting temperature, such as beryllium, aluminum or the metals of the rare earths, then, a deterioration of the vacuum during the working will no longer be noticed.

This effect, by far more favorable, as compared with that of the acids, may perhaps be explained by the fact that when the alkaline earth metals are generated according to the old process, certain alkaline earth combinations result, in addition to metal, such as the nitride, which are more or less of unstable character. Now it is decidedly possible, that these substances decompose under the influence of electrical discharges, and produce a deterioration of the vacuum, owing to the gases freed. On the other hand, the combinations produced by the generation of the metal of alkaline earth according to the novel process, such as the oxides of beryllium, aluminum and of the rare earths are known as substances, extremely difficult to decompose and as non-volatile, even when glowed. Thus they do not deteriorate the vacuum. It is however possible, that the different behavior of the tubes produced by both processes may be due to other reasons.

The reduction of the alkaline earth combinations according to the novel process is at times accompanied by an intense generation of heat, for instance when aluminum is used as a reducing medium, so that there is danger that together with the alkaline earth metal, noticeable quantities of the reducing medium also may vaporize. In these cases, it is advantageous to add to the mixture, suitable diluting means, such as beryllium oxide, aluminum oxide, as also metals volatilized with difficulty, such as tungsten, molybdenum, etc., and thus to avoid excessive heating during

55

60

65

70

75

80

85

90

95

100

the operation and a too rapid development of the vapor of the alkaline earth metal. Under circumstances, the diluting agents can even be added in excess.

The reaction can also be prolonged by employing mixtures of such substances, on which the reducing agents take effect in different degrees of intensity. For many purposes, good results have been attained by the employment, as diluting means, of metals which form alloys with the alkaline earth metals, such as aluminum, copper etc. From the alloy formed during the reaction, the alkaline earth metal, does not escape on glowing so quickly as it does from the pure mixture, in this manner, a current of metal vapor is attained of longer duration, which is of great advantage, for instance, for the production of oxide cathodes according to the alloying process mentioned in the introduction.

When employing oxides of alkaline earths, it has proved advantageous, to consolidate the mixture into blocks by pressure, and to protect the compressed blocks against the effect of water and carbonic acid by coating and saturating them with paraffin oil or similar liquids of sufficient viscosity, which have no effect on the mixture and which become volatile at a high temperature. These blocks are attached to the electrodes or to special carriers in suitable manner and the tubes sealed in, in known manner. The invention may be better understood by reference to the accompanying drawing in which the single figure is a side view partly in section of a radio tube adapted to be treated in accordance with the invention.

The radio tube comprises a bulb or envelope 1 having a stem 2 upon which is mounted in the usual way a cathode, such as a filament 3 surrounded by a grid 4 and a plate 5. A block 6 of the mixture containing the oxide of the desired alkaline earth metal may be mounted in various well known ways in suitable position, for example, on the plate 5 where it may be heated at will to cause evolution of the alkaline earth metal. A convenient way of heating the block 6 is by means of the high frequency coil commonly used in the art. After the tubes have been pumped out, the gas is extracted from the pressed blocks, advantageously by heating the same, for instance by high frequency or radiation heating to about 500° C. By slowly increasing the temperature to 700 to 800° C. the alkaline earth metal is vaporized and precipitated onto the walls or onto the cathodes. The further treatment takes place in the known manner.

In many cases it is usual to employ mixtures of oxides for oxide cathodes. According to the novel process such mixtures can be readily obtained, if, in the original mixture, the corresponding combinations of the alka-

line earth metals are selected as initial substances, for instance those of barium and strontium.

The new process enables an extremely rapid pumping out of the tubes, since, with the exception of the alkaline earth vapor, no gases are freed from the mixture introduced. The residue can have no deteriorating effect on the vacuum since it contains no decomposable substances. The metal of the alkaline earth developed, is of the highest purity and as a surface in the discharge tubes, it exceeds by far the gas clean-up effects of those metal surfaces which are produced by the old process.

Also in connection with tubes filled with rare gas, for instance the argon filled glow rectifiers in which the effect is soon deteriorated owing to the contents of nitrogen, the present process can be employed with advantage.

What I claim as new and desire to secure by Letters Patent of the United States, is:

The method of treating an electron discharge device having an evacuated envelope enclosing an anode and a cathode which comprises placing adjacent said cathode a mixture of an alkaline earth oxide, powdered aluminum, and a powdered refractory oxide non-reducible by aluminum and sufficient in amount to prolong the exothermic reaction between said alkaline earth oxide and aluminum, and heating said mixture to cause said reaction.

ERICH WIEGAND. 100

105

110

115

120

125

126